

Patented Nov. 17, 1925.

1,562,125

# UNITED STATES PATENT OFFICE.

WILLIAM H. RIDEOUT, OF PORTHILL, IDAHO.

## PROCESS FOR SEPARATING MOLYBDENUM FROM ITS ORE.

No Drawing.

Application filed March 13, 1924. Serial No. 699,146.

To all whom it may concern:

Be it known that I, WILLIAM H. RIDEOUT, a citizen of the United States, residing at Porthill, in the county of Boundary and 5 State of Idaho, have invented certain new and useful Improvements in Processes for Separating Molybdenum from Its Ore, of which the following is a specification.

This invention relates to means for separating molybdenum from its ores and the 10 primary object of the invention is the provision of a novel compound, which will, when the molybdenum bearing ore has been thoroughly ground up, effectively divide the 15 molybdenum from the ore and thus permit the easy separation of the molybdenum from the ore and the refining thereof.

Another object of the invention is the 20 provision of a novel method utilizing the improved compound for separating the molybdenum from the ore, the improved method reducing the cost and trouble of separating molybdenum from its ore to a minimum.

25 With these and other objects in view, the invention consists in the novel composition of ingredients, as will be now described.

In preparing the composition I prefer to 30 use the composition in about the following proportions: 90 gallons of water, 10 gallons of kerosene, 4 ounces of soda, and 1 pound of lye. The proportions of the ingredients relative to one another can be varied within certain limits, as will be hereinafter more 35 fully pointed out according to the richness of the molybdenum in the ore being refined, and whether the water is hard or soft. If the ore is rich in molybdenum I can use approximately 100 gallons of water 40 to 1 gallon of kerosene, but if the percentage of the molybdenum in the ore is very small I prefer to use 80 gallons of water to 20 gallons of kerosene. If the water used is hard I prefer to use one-half pound of soda and 45 2 pounds of lye to every 100 gallons of water, but if the water is soft I prefer to use one-half ounce of soda and one-quarter pound of lye to every 100 gallons of water.

50 In making the re-agent the water and kerosene are mixed thoroughly together after which the soda and lye are combined therewith. The lye and soda specified are potassium carbonate and bi-carbonate of soda respectively. The potassium carbonate 55 is preferably made from wood ashes.

In separating the molybdenum from the

ore, I prefer to use the following method, from which I found the best results can be obtained. The ore containing the molybdenum is thoroughly ground and reduced to 60 a powder by passing the same through any preferred type of reducing mill. The ore is preferably ground fine enough so that the same will pass through a 60 or 80 wire mesh screen. The ground-up ore is then 65 mixed with the water and agitated in the usual way and the resultant mixture or slime is passed through a series of vats so that the slime will settle to a certain extent. To this slime I add 2 gallons of improved 70 compound or re-agent to every gallon of the slime and the mixture is placed in a suitable vat and thoroughly agitated, after which the same is left to stand for a small 75 length of time so that dirt and the like can settle to the bottom. The oil, i. e., the re-agent, will float to the top carrying the molybdenum therewith and the oil and molybdenum are drawn off just below the 80 water line. The matter when drawn off is 85 passed through a filter and the re-agent will seep therethrough leaving the clean molybdenum on the filter. The re-agent can then be returned to the vat and the mass again 90 reagitated. This process is repeated two or three times until all of the molybdenum has been separated from the waste and other 95 metals contained in the ore.

From the foregoing description, it can 90 be seen that I have provided an exceptionally simple means by which I can effectively separate molybdenum from its ore.

Changes in detail may be made without 95 departing from the spirit or the scope of this invention.

What I claim as new is:

The method of separating molybdenum 100 from its ore consisting in reducing the ore to a fine mass, adding water to the mass to form a pulp, adding two gallons of a composition to every one gallon of the pulp, the composition being made in the following proportions: for every one hundred gallons, water ninety gallons, paraffin ten gallons, soda, four ounces, lye one pound, then 105 agitating the entire mixture, allowing the mixture to stand until the compound floats to the top thereof carrying the molybdenum therewith, and then withdrawing the compound and molybdenum from the mixture. 110

In testimony whereof I affix my signature.

WILLIAM H. RIDEOUT.